

## UNITED STATES PATENT OFFICE

CLIFFORD C. BUCHLER, OF CASPER, WYOMING, ASSIGNOR TO STANDARD OIL COMPANY, OF WHITING, INDIANA, A CORPORATION OF INDIANA

## HIGH MELTING POINT WAX

No Drawing.

Application filed March 5, 1928. Serial No. 259,373.

This invention relates to the production of high melting point waxes from petrolatum by filter pressing and sweating.

Heretofore it has not been possible to press and sweat petrolatum. The present invention is based upon the discovery that a petrolatum distillate containing a suitable amount of diluent may be readily pressed at appropriate temperatures to produce a filter cake 10 which can be satisfactorily sweated to a substantial yield of high melting point wax.

The distillation of the petrolatum ordinarily should be conducted at a temperature which will cause slight decomposition but excessive destruction of the high melting point wax should be prevented by conducting the distillation under conditions characteristic of sub-atmospheric distillation, that is, under vacuum or with steam or under vacuum with 20 steam. A substantial percentage of the petrolatum should be distilled over in order to ensure a good recovery of wax. Ordinarily the distillate is unpressable and requires to be diluted with a suitable amount of a petroleum distillate such as naphtha, to render it pressable. The addition of too much naphtha will render the wax unpressable, but the range of addition of naphtha which will ensure a pressable stock is broad and no difficulty is experienced in determining an 30 amount of naphtha to be added which will ensure satisfactory pressing. The amount of oil in the filter cake must be carefully regulated. If this oil-content is too high difficulties are experienced in pressing and sweating and the yield of sweated high melting point wax is seriously diminished. The oil-content of the filter cake is controlled by regulating the amount of diluent added and 40 the temperature of pressing. The oil-content of the wax cake diminishes with reduction of the amount of diluent and increases with the reduction of the pressing temperature.

45 To sum up, the process involves the addi-

tion of a quantity of diluent to the wax distillate which will ensure a pressable distillate and, in conjunction with the conditions of pressing, will ensure a filter cake of such low oil content that it can be readily sweated. 50

It is obvious that the conditions necessary for various wax distillates will vary considerably and that it is not possible to set forth specific figures which would be applicable to all distillates. However, I believe that satisfactory results can be obtained from most petrolatums by following the teaching of the appended specific example, with slight changes which may be necessitated for petrolatum distillates of somewhat different character. 55 60

*Example*

Petrolatum wax derived from the first centrifuging of a dilute and chilled reduced crude oil, and having a melting point of about 150° F. and an oil content of about 39%, is heated in a still to about 500° F. Steam is then supplied to the still and the temperature is rapidly raised to a maximum of about 800° 70 F. An overhead amounting to about 70% of the charge and having a melting point of about 122° F. and an oil-content of about 52%, is obtained. This overhead cannot be readily pressed but if it is diluted to give a stock 75 containing between about 10% and about 65% of naphtha it may be pressed without difficulty. I have found that for the wax distillate indicated the optimum content of naphtha is about 15%. The distillate thus diluted is chilled to about 74° F. and filter-pressed at a temperature of 74-78° F. The pressing occupies eight hours and the maximum pressure is about 120 lbs. per square inch. A yield of about 26% of wax cake is obtained, which contains about 8% naphtha and 8% of oil. I have found that the oil content should be controlled by the amount of dilution and temperature of pressing so that the oil content should preferably not exceed 10%, 80 85 90

in order to ensure a satisfactory sweating yield. The filter-cake has a melting point, after removal of naphtha of about 148° F. The filter-cake is subjected to sweating for 5 several days at a temperature rising from 110° F. to about 150° F., giving about 59% of wax containing about 1.5% of oil, having a melting point of 154° F. (155½ A. S. T. M.) and of good color. The yield is about 14% 10 of the initial petrolatum. The drips contain a substantial quantity of wax and may be readily resweated at slightly lower temperatures to give a substantial yield of wax of somewhat lower melting point.

15 By way of comparison it may be stated that on diluting similar distillate wax to a naphtha content of about 30% by weight and pressing between 67° and 70° F., a wax-cake containing about 14% of oil is obtained, while 20 if the pressing is effected at about 70° to 74° F., the oil content is about 11%. As illustrative of the effect of oil upon sweating, it may be stated that a composite wax thus obtained and containing about 12% of oil and 25 having a melting point of 144° F., after sweating over several days, with a temperature rising from 110° F. to 145½° F. gives a 48% yield of wax having a melting point of 150½° F. and an oil content about 7%.

30 Although the present invention has been described in connection with the details of a specific example, it must be understood that such details are not intended to be limitative upon the scope of the invention except 35 in so far as included in the accompanying claims.

I claim:

1. The method of producing high melting point wax from petrolatum wax which 40 consists in distilling the petrolatum wax under conditions characteristic of sub-atmospheric distillation, diluting the distillate with an oil miscible diluent and filter pressing the diluted distillate under temperature conditions 45 which give a sweatable cake, and sweating the filter cake.

2. The method of producing high melting point wax from petrolatum wax which 50 consists in distilling the petrolatum wax under conditions characteristic of sub-atmospheric distillation, diluting the wax distillate with low boiling petroleum distillate to form a diluted product containing between 10 and 55 65% of the petroleum distillate from which the wax may be readily pressed at a suitable pressing temperature, pressing the diluted wax distillate at such temperature, and sweating the filtered wax.

3. In the treatment of petrolatum wax, the 60 steps of distilling the petrolatum wax under conditions characteristic of sub-atmospheric distillation and diluting the wax distillate with a petroleum distillate to form a diluted product containing between 10 and 65% of 65 petroleum distillate from which pressable

wax may be separated by pressing the diluted distillate at suitable pressing temperatures.

4. The method of producing high melting point wax from petrolatum wax which consists in distilling the petrolatum wax under 70 conditions characteristic of sub-atmospheric distillation, diluting the distillate with petroleum distillate, and filter pressing the diluted distillate under temperature conditions which give a sweatable cake of relatively low 75 oil content, and sweating the filter cake.

5. The method of producing high melting point wax from petrolatum wax which consists in distilling the petrolatum wax under 80 conditions characteristic of sub-atmospheric distillation, diluting the wax distillate with low boiling petroleum diluent to form a product containing between 10 and 65% of petroleum diluent whereby such distillate is filter pressable at a suitable pressing temperature, 85 pressing the diluted wax distillate at such temperature, and sweating the filtered wax.

6. In the treatment of petrolatum wax, the steps of distilling the petrolatum wax under 90 conditions characteristic of sub-atmospheric distillation and diluting the wax distillate with a petroleum distillate to form a product containing between 10 and 65% of petroleum distillate which is filter pressable at suitable 95 pressing temperatures to give a cake of relatively low oil content.

7. The method of producing high melting point wax which consists in distilling petrolatum wax under conditions characteristic of sub-atmospheric distillation to obtain about 100 70% distillate, diluting the distillate to a naphtha content of about 15%, chilling the diluted distillate to about 74° F. and filtering at about 74 to 78° F., and sweating the separated wax.

8. The method of producing high melting point wax which consists in distilling petrolatum wax under conditions characteristic of sub-atmospheric distillation, diluting the wax distillate with petroleum distillate to 110 form a product containing between 10 and 65% of petroleum distillate whereby on cooling the distillate may be pressed to give a cake containing less than about 10% of oil, 115 pressing the diluted distillate to produce a cake containing less than about 10% of oil, and sweating the separated wax.

9. In the treatment of petrolatum wax, the steps of distilling the petrolatum wax under 120 conditions characteristic of sub-atmospheric distillation, diluting the wax distillate with an oil miscible diluent to form a product containing between 10 and 65% of the diluent, and cooling the diluted distillate to a temperature at which the wax may be separated 125 therefrom.

10. In the treatment of petrolatum wax, the steps of distilling the petrolatum wax under 130 conditions characteristic of sub-atmospheric distillation, diluting the wax distillate

with an oil miscible diluent to form a product containing between 10 and 65% of the diluent, cooling the diluted distillate to a temperature at which the wax may be separated 5 therefrom, separating the wax therefrom, and sweating the separated wax.

In testimony whereof, I have hereunto set my hand and seal this 1st day of March, 1928.

10 CLIFFORD C. BUCHLER.

15

20

25

30

35

40

45

50

55

60

65